

Nov. 19, 1940:

J. KNOEFEL

2,221,873

PRODUCTION OF MAT LIGHT-SENSITIVE PHOTOGRAPHIC PAPER

Filed Feb. 25, 1938



Fig. 1



Fig. 2



Fig. 3

INVENTOR  
Julius Knoefel  
BY *Shatz and John*  
HIS ATTORNEYS

## UNITED STATES PATENT OFFICE

2,221,873

PRODUCTION OF MAT LIGHT-SENSITIVE  
PHOTOGRAPHIC PAPER

Julius Knoefel, Leverkusen-Wiesdorf, Germany,  
assignor, by mesne assignments, to General Ani-  
line & Film Corporation, New York, N. Y., a cor-  
poration of Delaware

Application February 25, 1938, Serial No. 192,562  
In Germany March 16, 1937

7 Claims. (Cl. 95—8)

The present invention relates to improvements in producing mat light-sensitive photographic papers.

Among matting agents for light-sensitive photographic papers starch is the best known. Starch has, however, injurious properties which render the substitution for it of another matting agent highly desirable. The disadvantages of starch matting are associated both with the casting of the emulsion and the production of the image.

The chief disadvantage in casting is that the starch settles in the photographic emulsion, whereby streakiness and irregularities of all kinds are unavoidable in the matting.

A further disadvantage in the casting is that the paper receiving the emulsion becomes curved and rolled up during and after the drying process, so that the further use of it is made difficult.

In the production of the image the starch used as the matting agent has the disadvantage that the blacks of the photographic picture, especially with high degrees of matting, are grey and lack saturation, so that the gradation of the photographic picture is flat.

The aforesaid tendency of starch matted papers to roll up is not only a trouble in connection with the casting operation, but also very troublesome in the finished picture. In the usual hot drying of the starch matted picture the tendency of the starch to become paste gives rise to disturbing lustrous parts of the picture.

It is one of the objects of this invention to provide a process for minimizing or avoiding the foregoing and other disadvantages of the starch matting.

Another object is the provision of a process for matting photographic papers by means of a waxy material.

Still another object is to provide a process for producing mat photographic papers by adding wax or waxy material to the light-sensitive layer or the protective layer or both of these, the size of the particles of the added material exceeding that of the grain of the light-sensitive emulsion.

Further objects of the invention will appear from the detailed description following herein-after when taken with the accompanying self-explanatory drawing in which:

Figure 1 is a section through a film in which the light-sensitive layer carries a protective layer, both the sensitive layer and the protective layer containing wax particles;

Figure 2 is a section through a film of similar

construction excepting that the wax particles are in the sensitive layer only; and

Figure 3 is a similar section through a similar film wherein, however, the wax particles are confined to the protective layer.

The waxy substances hereinafter referred to generally as waxes solid at ordinary temperature do not settle in the photographic emulsion and do not produce either rolling up or curvature. In the finished picture the saturation of the blacks is not disadvantageously affected by the addition of wax nor is there a disturbing change in the gradation of the picture. The passage of the starch into paste with corresponding damage, during the hot drying of the photographic paper, need not be feared when waxy bodies are used.

It has already been proposed to add wax to a sensitive emulsion layer for the purpose of improving the mechanical properties of the layer. In that proposal, however, the size of the particles of wax is to be the same as that of the grain of the sensitive emulsion. The size of the grain of the waxy material may be brought to that desired by suitable methods of dispersion. In the process of this invention it is necessary that the dispersion of the wax, for instance in water, should have a sufficient stability so that the dispersion may be mixed in any desired proportion with the photographic emulsion without flocculation of the wax, with a proportion depending on the desired matting effect.

According to the invention dispersions of this kind can advantageously be obtained if, in the production of the aqueous dispersion of wax, both to the dispersing agent (water) and the body to be dispersed (wax) there is added before the dispersion an emulsifying agent. The emulsifying agents found in the market, for instance Saponin, Emulphor O (registered trade-mark), are suitable.

The following example illustrates the invention:

15 grams of montana wax, 5 grams of stearic acid and 2.5 grams of Emulphor O are melted together on the water bath. 2.5 grams of Emulphor O are dissolved in 100 cc. of water and while stirring at 80° C. the molten mixture of wax is poured into the solution. The aqueous dispersion of wax thus obtained is then cooled and added to the photographic emulsion. The size of the particles in the dispersion is considerably larger than that of the silver-halide grain in the usual photographic paper emulsion.

In the example the montana wax and the

stearic acid may be exchanged for a ceresin wax, carnauba wax, a synthetic wax, fatty acids of high molecular weight and other waxy bodies.

What I claim is:

- 5 1. A photographic paper comprising in superimposition a paper support, a silver halide emulsion layer and a protective layer, at least one of said layers containing a wax solid at ordinary temperature, the size of the particles of said substance exceeding that of the grain of said emulsion layer.
- 10 2. A photographic paper comprising in superimposition a paper support, a silver halide emulsion layer and a protective layer, said emulsion layer containing a wax solid at ordinary temperature, the size of the particles of said substance exceeding that of the grain of said emulsion layer.
- 15 3. A photographic paper comprising in superimposition a paper support, a silver halide emulsion layer and a protective layer, said protective layer containing a wax solid at ordinary temperature, the size of the particles of said substance exceeding that of the grain of said emulsion layer.
- 20 4. A photographic paper comprising in superimposition a paper support, a silver halide emulsion layer and a protective layer, said emulsion layer containing a wax solid at ordinary temperature, the size of the particles of said substance exceeding that of the grain of said emulsion layer.
- 25 5. A photographic paper comprising in superimposition a paper support, a silver halide emulsion layer and a protective layer, at least one of said layers containing montana wax, the size of the particles of said substance exceeding that of the grain of said emulsion layer.
6. A photographic paper comprising in superimposition a paper support, a silver halide emulsion layer and a protective layer, at least one of said layers containing a synthetic wax, the size of the particles of said substance exceeding that of the grain of said emulsion layer.
- 10 7. A photographic paper comprising in superimposition a paper support, a silver halide emulsion layer and a protective layer, at least one of said layers containing a fatty acid of high molecular weight, the size of the particles of said substance exceeding that of the grain of said emulsion layer.

25

JULIUS KNOEFEL.